



US009832818B2

(12) **United States Patent**  
**Decker et al.**

(10) **Patent No.:** **US 9,832,818 B2**  
(45) **Date of Patent:** **Nov. 28, 2017**

(54) **RESISTIVE HEATING COATINGS  
CONTAINING GRAPHENIC CARBON  
PARTICLES**

(71) Applicant: **PPG Industries Ohio, Inc.**, Cleveland, OH (US)

(72) Inventors: **Eldon L. Decker**, Gibsonia, PA (US); **Noel R. Vanier**, Wexford, PA (US); **John M. Furar**, Pittsburgh, PA (US); **Stephen B. Istivan**, Pittsburgh, PA (US); **Cheng-Hung Hung**, Wexford, PA (US)

(73) Assignee: **PPG Industries Ohio, Inc.**, Cleveland, OH (US)

(\*) Notice: Subject to any disclaimer, the term of this patent is extended or adjusted under 35 U.S.C. 154(b) by 0 days.

(21) Appl. No.: **14/529,786**

(22) Filed: **Oct. 31, 2014**

(65) **Prior Publication Data**

US 2015/0053668 A1 Feb. 26, 2015

**Related U.S. Application Data**

(63) Continuation-in-part of application No. 14/337,427, filed on Jul. 22, 2014, now Pat. No. 9,475,946, which (Continued)

(51) **Int. Cl.**

**H05B 3/14** (2006.01)  
**H05B 3/26** (2006.01)  
**H05B 3/34** (2006.01)

(52) **U.S. Cl.**

CPC ..... **H05B 3/145** (2013.01); **H05B 3/26** (2013.01); **H05B 3/34** (2013.01); (Continued)

(58) **Field of Classification Search**  
CPC ..... H05B 3/14  
See application file for complete search history.

(56) **References Cited**

**U.S. PATENT DOCUMENTS**

4,851,262 A 7/1989 McFeaters  
5,486,675 A 1/1996 Taylor et al.  
(Continued)

**FOREIGN PATENT DOCUMENTS**

CN 102877109 A 1/2013  
CN 103468057 A 12/2013  
(Continued)

**OTHER PUBLICATIONS**

Kang, Junmo et al., "High-Performance Graphene-Based Transparent Flexible Heaters", Nano Letters; Dec. 14, 2011; pp. 5154-5158; vol. 11, No. 12; ACS Publications, American Chemical Society.

(Continued)

*Primary Examiner* — Daniel C McCracken

(74) *Attorney, Agent, or Firm* — Alan G. Towner

(57) **ABSTRACT**

Resistive heating assemblies comprising a substrate, a conductive coating comprising graphenic carbon particles applied to at least a portion of the substrate, and a source of electrical current connected to the conductive coating are disclosed. Conductive coatings comprising graphenic carbon particles having a thickness of less than 100 microns and an electrical conductivity of greater than 10,000 S/m are also disclosed.

**22 Claims, 5 Drawing Sheets**

5  
2



## Related U.S. Application Data

is a continuation-in-part of application No. 14/100, 064, filed on Dec. 9, 2013, now Pat. No. 9,574,094, and a continuation-in-part of application No. 14/348, 280, filed as application No. PCT/US2012/057811 on Sep. 28, 2012, now Pat. No. 9,221,688, which is a continuation-in-part of application No. 13/249,315, filed on Sep. 30, 2011, now Pat. No. 8,486,363, and a continuation-in-part of application No. 13/309,894, filed on Dec. 2, 2011, now Pat. No. 8,486,364.

## (52) U.S. Cl.

CPC .. H05B 2203/011 (2013.01); H05B 2203/013 (2013.01); H05B 2214/04 (2013.01)

## (56)

## References Cited

## U.S. PATENT DOCUMENTS

|                 |         |                      |
|-----------------|---------|----------------------|
| 5,527,518 A     | 6/1996  | Lynum et al.         |
| 5,749,937 A     | 5/1998  | Detering et al.      |
| 5,763,548 A     | 6/1998  | Matyjaszewski et al. |
| 5,788,738 A     | 8/1998  | Pirzada et al.       |
| 5,789,487 A     | 8/1998  | Matyjaszewski et al. |
| 5,807,937 A     | 9/1998  | Matyjaszewski et al. |
| 5,851,507 A     | 12/1998 | Pirzada et al.       |
| 5,935,293 A     | 8/1999  | Detering et al.      |
| 5,984,997 A     | 11/1999 | Bickmore et al.      |
| 5,989,648 A     | 11/1999 | Phillips             |
| 6,099,696 A     | 8/2000  | Schwob et al.        |
| 6,228,904 B1    | 5/2001  | Yadav et al.         |
| 6,316,119 B1    | 11/2001 | Metzger et al.       |
| 6,358,375 B1    | 3/2002  | Schwob               |
| 6,441,066 B1    | 8/2002  | Woodworth et al.     |
| RE37,853 E      | 9/2002  | Detering et al.      |
| 6,652,967 B2    | 11/2003 | Yadav et al.         |
| 6,669,823 B1    | 12/2003 | Sarkas et al.        |
| 6,689,192 B1    | 2/2004  | Phillips et al.      |
| 6,716,525 B1    | 4/2004  | Yadav et al.         |
| 6,719,821 B2    | 4/2004  | Yadav et al.         |
| 6,786,950 B2    | 9/2004  | Yadav et al.         |
| 6,821,500 B2    | 11/2004 | Fincke et al.        |
| 6,830,822 B2    | 12/2004 | Yadav                |
| 6,849,109 B2    | 2/2005  | Yadav et al.         |
| 7,071,258 B1    | 7/2006  | Jang et al.          |
| 7,635,458 B1    | 12/2009 | Hung et al.          |
| 7,754,184 B2    | 7/2010  | Mercuri              |
| 7,776,303 B2    | 8/2010  | Hung et al.          |
| 7,785,492 B1    | 8/2010  | Jang et al.          |
| 7,790,285 B2    | 9/2010  | Zhamu et al.         |
| 7,824,741 B2    | 11/2010 | Sandhu               |
| 7,842,271 B2    | 11/2010 | Petrik               |
| 8,047,248 B2    | 11/2011 | Prud'homme et al.    |
| 8,048,950 B2    | 11/2011 | Prud'homme et al.    |
| 8,129,466 B2    | 3/2012  | Polk et al.          |
| 8,486,363 B2    | 7/2013  | Hung et al.          |
| 8,486,364 B2    | 7/2013  | Vanier et al.        |
| 2002/0114949 A1 | 8/2002  | Bower et al.         |
| 2004/0247515 A1 | 12/2004 | Gardner              |
| 2005/0271574 A1 | 12/2005 | Jang et al.          |
| 2006/0093885 A1 | 5/2006  | Krusic et al.        |
| 2006/0121279 A1 | 6/2006  | Petrik               |
| 2006/0216222 A1 | 9/2006  | Jang                 |
| 2007/0045116 A1 | 3/2007  | Hung et al.          |
| 2007/0096066 A1 | 5/2007  | Yoshida et al.       |
| 2007/0237705 A1 | 10/2007 | Itoh et al.          |
| 2008/0206124 A1 | 8/2008  | Jang et al.          |
| 2009/0022649 A1 | 1/2009  | Zhamu et al.         |
| 2009/0054581 A1 | 2/2009  | Prud'homme et al.    |
| 2009/0068471 A1 | 3/2009  | Choi et al.          |
| 2009/0075035 A1 | 3/2009  | O'Brien et al.       |
| 2009/0110627 A1 | 4/2009  | Choi et al.          |
| 2009/0169467 A1 | 7/2009  | Zhamu et al.         |
| 2010/0036023 A1 | 2/2010  | Weng et al.          |
| 2010/0047154 A1 | 2/2010  | Lee et al.           |

|                  |         |                   |
|------------------|---------|-------------------|
| 2010/0055017 A1  | 3/2010  | Vanier et al.     |
| 2010/0055025 A1  | 3/2010  | Jang et al.       |
| 2010/0072430 A1  | 3/2010  | Gergely et al.    |
| 2010/0096597 A1  | 4/2010  | Prud'homme et al. |
| 2010/0126660 A1  | 5/2010  | O'Hara            |
| 2010/0247801 A1  | 9/2010  | Zenasni           |
| 2010/0255219 A1  | 10/2010 | Wenxu et al.      |
| 2010/0301212 A1  | 12/2010 | Dato et al.       |
| 2010/0303706 A1  | 12/2010 | Wallace et al.    |
| 2010/0314788 A1  | 12/2010 | Hung et al.       |
| 2010/0323113 A1  | 12/2010 | Ramappa et al.    |
| 2011/0046289 A1  | 2/2011  | Zhamu et al.      |
| 2011/0070426 A1  | 3/2011  | Vanier et al.     |
| 2012/0012796 A1  | 1/2012  | Chen et al.       |
| 2012/0021160 A1  | 1/2012  | Kariyada          |
| 2012/0142832 A1  | 6/2012  | Varma et al.      |
| 2012/0208008 A1* | 8/2012  | Tour .....        |
|                  |         | B82Y 30/00        |
|                  |         | 428/336           |
| 2012/0211160 A1  | 8/2012  | Asay et al.       |
| 2012/0277360 A1  | 11/2012 | Scheffer et al.   |
| 2012/0302683 A1* | 11/2012 | Ku .....          |
|                  |         | C09C 1/44         |
|                  |         | 524/186           |
| 2013/0084237 A1* | 4/2013  | Vanier .....      |
|                  |         | B82Y 30/00        |
|                  |         | 423/448           |
| 2015/0015902 A1  | 1/2015  | Feng              |
| 2015/0053668 A1* | 2/2015  | Decker .....      |
|                  |         | H05B 3/145        |
|                  |         | 219/553           |

## FOREIGN PATENT DOCUMENTS

|    |                 |              |
|----|-----------------|--------------|
| DE | 102010038079 A1 | 4/2012       |
| DE | 102011003619 A1 | 8/2012       |
| EP | 2562766 A1      | 2/2013       |
| KR | 20130013689 A   | 2/2012       |
| KR | 20120029530 A   | 3/2012       |
| WO | 1998040415 A1   | 9/1998       |
| WO | 2004/03096 A1   | 1/2004       |
| WO | 2004003096 A1   | 1/2004       |
| WO | 2009134492 A2   | 11/2009      |
| WO | 2010107769 A2   | 9/2010       |
| WO | 2011012874 A1   | 2/2011       |
| WO | 2011086391 A1   | 7/2011       |
| WO | 2013049498 A1   | 4/2013       |
| WO | 2013165677 A1   | 11/2013      |
| WO | 2013166414 A2   | 11/2013      |
| WO | 2013192180 A2   | 12/2013      |
| WO | 2014070346 A1   | 5/2014       |
| WO | 2014/076259 *   | 5/2014 ..... |
| WO | 2015089026 A1   | 6/2015       |
|    |                 | H01M 4/60    |

## OTHER PUBLICATIONS

Bergeron, Emmanuel "Production of Carbon by Pyrolysis of Methane in Thermal Plasma", Master's Thesis in Applied Sciences, University of Sherbrooke, Faculty of Applied Sciences, Department of Chemical Engineering, Quebec, Canada, Oct. 1997.

Cassagneau et al., "Preparation of Layer-by-Layer Self-Assembly of Silver Nanoparticles Capped by Graphite Oxide Nanosheets", *J. Phys. Chem. B* 1999, 103, 1789-1793.

Chen, Shanshan et al. "Oxidation Resistance of Graphene-Coated Cu and Cu/Ni Alloy", *ACS Nano*, Jan. 28, 2011, pp. 1321-1327.

Choi, Ki Seok et al. "Fabrication of Free-Standing Multilayered Graphene and Poly(3,4-ethylenedioxythiophene) Composite Films with Enhanced Conductive and Mechanical Properties", *Langmuir*, 26 (15), 2010, pp. 12902-12908.

Coraux, Johann "Growth of Graphene on Ir(111)", *New Journal of Physics* 11, 2009, 023006, pp. 1-22.

Dato, Albert et al. "Substrate-Free Gas-Phase Synthesis of Graphene Sheets", *Nano Letters*, vol. 8, No. 7, 2008, pp. 2012-2016.

Dresselhaus et al., *Science of Fullerenes and Carbon Nanotubes*, pp. 60-79 (Academic Press 1996).

Du, X.S. et al. "Facile Synthesis of Highly Conductive Polyaniline/Graphite Nanocomposites" *European Polymer Journal* 40, 2000, pp. 1489-1493.

Fincke, James R. et al. "Plasma Pyrolysis of Methane to Hydrogen and Carbon Black" *Ind. Eng. Chem. Res.*, 2002, pp. 1425-1435.

(56)

## References Cited

## OTHER PUBLICATIONS

- Fitzer et al., Recommended Terminology for the Description of Carbon as a Solid, *Pure & Appl. Chem.* 1995; 67(3): 473-506.
- Gannon, Richard E. "Acetylene from Hydrocarbons", Kirk-Othmer Encyclopedia of Chemical Technology, 2003, pp. 1-28.
- Gomez De Arco, Lewis et al. "Synthesis, Transfer, and Devices of Single- and Few-Layer Graphene by Chemical Vapor Deposition", *IEEE Transactions on Nanotechnology*, Vo. 8, No. 2, Mar. 2009, pp. 135-138.
- Gonzalez-Aguilar, J. et al. "Carbon Nanostructures Production by Gas-Phase Plasma Processes at Atmospheric Pressure", *J. Phys. D: Appl. Phys.* 40, 2007, pp. 2361-2374.
- Holmen, A. et al. "High-Temperature Pyrolysis of Hydrocarbons. 1. Methane to Acetylene", *The Norwegian Institute of Technology*, University of Trondheim, Ind. Eng. Chem., Process Des. Dev., vol. 15, No. 3, 1976.
- Ji, Liwen et al. "Graphene/Si Multilayer Structure Anodes for Advanced Half and Full Lithium-Ion Cells", *Nano Energy*, 2011.
- Khan, M.S. et al. "Survey of Recent Methane Pyrolysis Literature", *Industrial and Engineering Chemistry*, vol. 62, No. 10, Oct. 1970.
- Kim, Juhan et al. "Fabrication of Graphene Flakes Composed of Multi-Layer Graphene Sheets using a Thermal Plasma Jet System", *Nanotechnology* 21, Jan. 29, 2010.
- Kim, Keun Su et al. "Continuous Synthesis of Nanostructured Sheetlike Carbons by Thermal Plasma Decomposition of Methane", *IEEE Transactions on Plasma Science*, vol. 35, No. 2, Apr. 2007.
- Kirk-Othmer Encyclopedia of Chemical Technology, "Acetylene From Hydrocarbons", pp. 1-28.
- Kostic et al., "Thermodynamic Consideration of B-O-C-H System for Boron Carbide (B4C) Powder Synthesis in Thermal Plasma", 1997, *Progress in Plasma Processing of Materials*, pp. 889-898.
- Lavoie, Martin "Synthesis of Carbon Black From Propane Using a Thermal Plasma", Master's Thesis in Applied Sciences, University of Sherbrooke, Faculty of Applied Sciences, Department of Chemical Engineering, Quebec, Canada, Sep. 1997.
- Malesevic, Alexander et al. "Synthesis of Few-Layer Graphene Via Microwave Plasma-Enhanced Chemical Vapour Deposition", *Nanotechnology* 19, 2008, 305604 (6pps).
- Martin-Gallego, M. et al. "Epoxy-Graphene UV-Cured Nanocomposites", *Polymer* 52, 2011, pp. 4664-4669.
- McWilliams, Andrew, "Market Research Report, Graphene: Technologies, Applications, and Markets", BCC Research, Feb. 2011.
- Nandamuri, G. et al. "Chemical Vapor Deposition of Graphene Films" *Nanotechnology* 21, 2010, 145604 (4pp).
- Prasai, Dhiraj et al. "Graphene: Corrosion-Inhibiting Coating" *ACS Nano*, 6 (2), 2012, pp. 1102-1108.
- Pristavita, Ramona et al. "Carbon Blacks Produced by Thermal Plasma: the Influence of the Reactor Geometry on the Product Morphology", *Plasma Chem Plasma Process*, 30, 2010, pp. 267-279.
- Pristavita, Ramona et al. "Carbon Nanoparticle Production by Inductively Coupled Thermal Plasmas: Controlling the Thermal History of Particle Nucleation" *Plasma Chem Plasma Process*, 31, 2011, pp. 851-866.
- Pristavita, Ramona et al., "Carbon Nano-Flakes Produced by an Inductively Coupled Thermal Plasma System for Catalyst Applications", *Plasma Chem Plasma Process*, 31, 2011, pp. 393-403.
- Skinner, Gordon B. "Pyrolysis of Methane and the C2 Hydrocarbons", Monsanto Chemical Co., Research and Engineering Division, Dayton 7, Ohio, pp. 59-68.
- Su, Fang-Yuan et al. "Could Graphene Construct an Effective Conducting Network in a High-Power Lithium Ion Battery?" *Nano Energy*, Feb. 25, 2012.
- Subrahmanyam, K.S. et al. "Simple Method of Preparing Graphene Flakes by an Arc-Discharge Method", *The Journal of Physical Chemistry C*, vol. 113, No. 11, 2009, pp. 4257-4259.
- Tang et al., "Processible Nanostructured Materials with Electrical Conductivity and Magnetic Susceptibility: Preparation and Properties of Maghemite/Polyaniline Nanocomposite Films", *Chem. Mater.* 1999, 11, 1581-1589.
- Zhong, Ziyi et al. "Catalytic Growth of Carbon Nanoballs With and Without Cobalt Encapsulation", *Chemical Physics Letters* 330, 2000, pp. 41-47.

\* cited by examiner



FIG. 1



FIG. 2



FIG. 3



FIG. 4



FIG. 5

## 1

**RESISTIVE HEATING COATINGS  
CONTAINING GRAPHENIC CARBON  
PARTICLES**

**CROSS REFERENCE TO RELATED  
APPLICATIONS**

This application is a continuation-in-part of U.S. patent application Ser. No. 14/337,427 filed Jul. 22, 2014, which is both a continuation-in-part of U.S. patent application Ser. No. 14/100,064 filed Dec. 9, 2013, and a continuation-in-part of U.S. patent application Ser. No. 14/348,280 filed Mar. 28, 2014. U.S. patent application Ser. No. 14/348,280 is a 371 national stage entry of PCT/US2012/057811 filed Sep. 28, 2012, which is a continuation-in-part U.S. patent application Ser. No. 13/249,315 filed Sep. 30, 2011, now U.S. Pat. No. 8,486,363 issued Jul. 16, 2013, and is also a continuation-in-part of U.S. patent application Ser. No. 13/309,894 filed Dec. 2, 2011, now U.S. Pat. No. 8,486,364 issued Jul. 16, 2013, all of which are incorporated herein by reference.

**FIELD OF THE INVENTION**

The present invention relates to resistive heating coatings containing graphenic carbon particles.

**BACKGROUND OF THE INVENTION**

Heated panels have many potential uses in various industries such as architecture, consumer products, automotive and aircraft industries and the like.

**SUMMARY OF THE INVENTION**

An aspect of the invention provides a resistive heating assembly comprising: a substrate; a conductive coating comprising graphenic carbon particles applied to at least a portion of the substrate, and a source of electrical current connected to the conductive coating.

Another aspect of the invention provides a conductive coating comprising graphenic carbon particles having a thickness of less than 100 microns and an electrical conductivity of greater than 10,000 S/m.

**BRIEF DESCRIPTION OF THE DRAWINGS**

FIG. 1 is a partially schematic sectional isometric view of a resistive heating coating applied on a substrate in accordance with an embodiment of the present invention.

FIG. 2 is a partially schematic top view of a test panel for measuring heating rates of various coatings.

FIG. 3 is a graph of temperature versus time for two resistively heated coatings.

FIG. 4 is a partially schematic top view of a test panel for measuring heating rates of various coatings.

FIG. 5 is a graph of temperature versus time for three resistively heated coatings.

**DETAILED DESCRIPTION OF EMBODIMENTS  
OF THE INVENTION**

In accordance with embodiments of the present invention, graphenic carbon particles are used in coatings to provide increased electrical conductivity and the ability to serve as

## 2

resistive heating coatings. Such coatings may have relatively small thicknesses while exhibiting desirable resistive heating properties.

The resistive heating coatings of the present invention have many potential applications, such as architectural coatings, industrial coatings, automotive seat warmers, clothing and the like. In architectural applications, the coatings may be applied to walls, ceilings, floors, and the like to provide heating for commercial and residential buildings. In industrial applications, the resistive heating coatings may be applied to aircraft for deicing, ice-prevention, shape controlling or other purposes, automotive vehicle panels, mirrors or other components for deicing or anti-fogging purposes.

As used herein, the term "electrically conductive", when referring to a coating containing graphenic carbon particles, means that the coating has an electrical conductivity of at least 0.001 S/m. For example, the coating may have a conductivity of at least 0.01, or at least 10 S/m. When the electrically conductive coating is used in a resistive heating assembly in accordance with embodiments of the invention, the conductivity may typically be from 10,000 to 50,000 S/m, or higher. In certain embodiments, the conductivity may be at least 12,000 S/m or at least 20,000 S/m. For example, the conductivity may be at least 30,000 S/m, or at least 40,000 S/m, or at least 50,000 S/m or higher, or at least 60,000 S/m or higher.

In accordance with certain embodiments, the coatings do not exhibit significant electrical conductivity absent the addition of graphenic carbon particles. For example, a cured or dried polymeric resin may have a conductivity that is not measurable, while cured or dried polymeric resins of the present invention including graphenic carbon particles may exhibit conductivities as noted above.

As used herein, the term "coating" means any type of film having a measurable thickness when applied to a substrate. In certain embodiments, the coating may include a film-forming resin, may be free of a film-forming resin, or may be provided in the form of an ink.

As used herein, the term "resistive heating coating" means a coating which is heated by means of applying a voltage to the coating. This is also known as Joule heating or ohmic heating, where the electrical power dissipated in the coating is equal to  $I^2R$  where  $I$  is the current flow in the coating due to the applied voltage, and  $R$  is electrical resistance of the coating. Such resistive heating coatings may be applied to various different types of rigid or flexible substrates such as metal, glass, plastic, ceramic, composite, fabric and the like. Voltage may be selectively applied to such coatings by any suitable means, such as by electrically conductive contacts, wires or printed strips located on opposite edges of the coating that create an electric potential causing current to flow through the coating from one electrical contact to the other, e.g., in the plane of the coating.

FIG. 1 schematically illustrates a resistive heating coating 10 applied on a substrate 12 in accordance with an embodiment of the present invention. Electrical contacts 14 are provided on opposite edges of the coating 10. A conventional applied voltage (not shown) may be connected to the electrical contacts 14 to generate a flow of electric current  $I$  through the coating 10. The coating 10 has a thickness  $T$ . In certain embodiments, the coating 10 has a typical thickness  $T$  of from 0.1 to 100 microns, for example, from 1 to 50 microns or from 5 to 25 microns. The coatings may be relatively thin while providing desirable resistive heating characteristics due to the electrical conductivity properties provided by the graphenic carbon particles. In certain

embodiments, the thin coatings are sufficiently flexible such that they do not suffer damage when applied to flexible substrates.

FIGS. 2 and 4 schematically illustrate resistive heating assemblies in the form of test panels in accordance with embodiments of the present invention. In FIG. 2, the resistive heating test panel includes a resistive heating coating 110 applied on a glass substrate 112. Electrically conductive wires 114 are connected at opposite ends of the resistive heating coating 110 by adhesive 116. In FIG. 4, the resistive heating test panel includes a resistive heating coating 210 applied on a metal substrate 212. Electrically conductive wires 214 are connected at opposite ends of the resistive heating coating 210 by adhesive 216.

In certain embodiments, a single type of graphenic carbon particles may be dispersed in the coatings. In other embodiments, co-dispersions of different types of graphenic particles may be used. As used herein, the term "co-dispersed" means that different types of graphenic carbon particles are dispersed together in a medium such as a solvent containing a polymeric dispersant to form a substantially uniform dispersion of the graphenic carbon particles throughout the medium without substantial agglomeration of the particles. As used herein, the term "mixture" means that different types of graphenic carbon particles are dispersed separately in a medium, followed by mixing the separate dispersions together. The presence of agglomerations may be determined by standard methods such as visual analysis of TEM micrograph images. Agglomerations may also be detected by standard particle size measurement techniques, as well as measurements of electrical conductivity or measurements of optical characteristics of materials containing the graphenic carbon particles such as color, haze, jetness, reflectance and transmission properties. The different types of graphenic particles that are dispersed together may comprise particles having different particle size distributions, thicknesses, aspect ratios, structural morphologies, edge functionalities and/or oxygen contents. In certain embodiments, the graphenic carbon particles are made by different processes, such as thermal production methods, exfoliation methods, and the like, as more fully described below.

In certain embodiments, the graphenic carbon particles may be dispersed within a matrix material such as a film-forming resin, a dispersant or a mixture of dispersants in amounts of from 0.1 to 95 weight percent based on the total solids of the material. For example, the graphenic carbon particles may comprise from 1 to 90 weight percent, or from 5 to 85 weight percent of the material. In certain embodiments, the amount of graphenic carbon particles contained in the materials may be relatively large, such as from 40 or 50 weight percent up to 90 or 95 weight percent. For example, the graphenic carbon particles may comprise from 60 to 85 weight percent, or from 70 to 80 weight percent. In certain embodiments, conductivity properties of ink or coating may be significantly increased with relatively minor additions of the graphenic carbon particles, for example, less than 50 weight percent, or less than 30 weight percent. In certain embodiments, the coatings or other materials have sufficiently high electrical conductivities at relatively low loadings of the graphenic carbon particles. For example, the above-noted electrical conductivities may be achieved at graphenic carbon particle loadings of less than 20 or 15 weight percent. In certain embodiments, the particle loadings may be less than 10 or 8 weight percent, or less than 6 or 5 weight percent. For example, for coatings comprising film-forming polymers or resins that by themselves are non-conductive, the dispersion of from 3 to 5 weight percent

of graphenic carbon particles may provide an electrical conductivity of at least 0.1 S/m, e.g., or at least 10 S/m.

The compositions can comprise any of a variety of thermoplastic and/or thermosetting compositions known in the art. For example, the coating compositions can comprise film-forming resins selected from epoxy resins, acrylic polymers, polyester polymers, polyurethane polymers, polyamide polymers, polyether polymers, bisphenol A based epoxy polymers, polysiloxane polymers, styrenes, ethylenes, butylenes, copolymers thereof, and mixtures thereof. Generally, these polymers can be any polymers of these types made by any method known to those skilled in the art. Such polymers may be solvent borne, water soluble or water dispersible, emulsifiable, or of limited water solubility. Furthermore, the polymers may be provided in sol gel systems, may be provided in core-shell polymer systems, or may be provided in powder form. In certain embodiments, the polymers are dispersions in a continuous phase comprising water and/or organic solvent, for example emulsion polymers or non-aqueous dispersions.

In addition to the resin and graphenic carbon particle components, the coatings or other materials in accordance with certain embodiments of the present invention may include additional components conventionally added to coating or ink compositions, such as cross-linkers, pigments, tints, flow aids, defoamers, dispersants, solvents, UV absorbers, catalysts and surface active agents. In certain embodiments, the coatings may be colored, while in other embodiments the coatings may be clear.

Thermosetting or curable coating compositions typically comprise film forming polymers or resins having functional groups that are reactive with either themselves or a cross-linking agent. The functional groups on the film-forming resin may be selected from any of a variety of reactive functional groups including, for example, carboxylic acid groups, amine groups, epoxide groups, hydroxyl groups, thiol groups, carbamate groups, amide groups, urea groups, isocyanate groups (including blocked isocyanate groups and tri-alkylcarbamoyltriazine) mercaptan groups, styrenic groups, anhydride groups, acetoacetate acrylates, uretidione and combinations thereof.

Thermosetting coating compositions typically comprise a crosslinking agent that may be selected from, for example, aminoplasts, polyisocyanates including blocked isocyanates, polyepoxides, beta-hydroxyalkylamides, polyacids, anhydrides, organometallic acid-functional materials, polyamines, polyamides, and mixtures of any of the foregoing. Suitable polyisocyanates include multifunctional isocyanates. Examples of multifunctional polyisocyanates include aliphatic diisocyanates like hexamethylene diisocyanate and isophorone diisocyanate, and aromatic diisocyanates like toluene diisocyanate and 4,4'-diphenylmethane diisocyanate. The polyisocyanates can be blocked or unblocked. Examples of other suitable polyisocyanates include isocyanurate trimers, allophanates, and uretdiones of diisocyanates. Examples of commercially available polyisocyanates include DESMODUR N3390, which is sold by Bayer Corporation, and TOLONATE HDT90, which is sold by Rhodia Inc. Suitable aminoplasts include condensates of amines and/or amides with aldehyde. For example, the condensate of melamine with formaldehyde is a suitable aminoplast. Suitable aminoplasts are well known in the art. A suitable aminoplast is disclosed, for example, in U.S. Pat. No. 6,316,119 at column 5, lines 45-55, incorporated by reference herein. In certain embodiments, the resin can be self crosslinking. Self crosslinking means that the resin contains functional groups that are capable of reacting with

themselves, such as alkoxy silane groups, or that the reaction product contains functional groups that are coreactive, for example hydroxyl groups and blocked isocyanate groups.

The dry film thickness of the cured coatings may typically range from less than 0.5 microns to 100 microns or more, for example, from 1 to 50 microns. As a particular example, the cured coating thickness may range from 1 to 15 microns. However, significantly greater coating thicknesses, and significantly greater material dimensions for non-coating materials, are within the scope of the invention.

As used herein, the term "graphenic carbon particles" means carbon particles having structures comprising one or more layers of one-atom-thick planar sheets of  $sp^2$ -bonded carbon atoms that are densely packed in a honeycomb crystal lattice. The average number of stacked layers may be less than 100, for example, less than 50. In certain embodiments, the average number of stacked layers is 30 or less, such as 20 or less, 10 or less, or, in some cases, 5 or less. The graphenic carbon particles may be substantially flat, however, at least a portion of the planar sheets may be substantially curved, curled, creased or buckled. The particles typically do not have a spheroidal or equiaxed morphology.

In certain embodiments, the graphenic carbon particles have a thickness, measured in a direction perpendicular to the carbon atom layers, of no more than 10 nanometers, no more than 5 nanometers, or, in certain embodiments, no more than 4 or 3 or 2 or 1 nanometers, such as no more than 3.6 nanometers. In certain embodiments, the graphenic carbon particles may be from 1 atom layer up to 3, 6, 9, 12, 20 or 30 atom layers thick, or more. In certain embodiments, the graphenic carbon particles have a width and length, measured in a direction parallel to the carbon atoms layers, of at least 50 nanometers, such as more than 100 nanometers, in some cases more than 100 nanometers up to 500 nanometers, or more than 100 nanometers up to 200 nanometers. The graphenic carbon particles may be provided in the form of ultrathin flakes, platelets or sheets having relatively high aspect ratios (aspect ratio being defined as the ratio of the longest dimension of a particle to the shortest dimension of the particle) of greater than 3:1, such as greater than 10:1.

In certain embodiments, the graphenic carbon particles have relatively low oxygen content. For example, the graphenic carbon particles may, even when having a thickness of no more than 5 or no more than 2 nanometers, have an oxygen content of no more than 2 atomic weight percent, such as no more than 1.5 or 1 atomic weight percent, or no more than 0.6 atomic weight, such as about 0.5 atomic weight percent. The oxygen content of the graphenic carbon particles can be determined using X-ray Photoelectron Spectroscopy, such as is described in D. R. Dreyer et al., Chem. Soc. Rev. 39, 228-240 (2010).

In certain embodiments, the graphenic carbon particles have a B.E.T. specific surface area of at least 50 square meters per gram, such as 70 to 1000 square meters per gram, or, in some cases, 200 to 1000 square meters per grams or 200 to 400 square meters per gram. As used herein, the term "B.E.T. specific surface area" refers to a specific surface area determined by nitrogen adsorption according to the ASTM D 3663-78 standard based on the Brunauer-Emmett-Teller method described in the periodical "The Journal of the American Chemical Society", 60, 309 (1938).

In certain embodiments, the graphenic carbon particles have a Raman spectroscopy 2D/G peak ratio of at least 1:1, for example, at least 1.2:1 or 1.3:1. As used herein, the term

"2D/G peak ratio" refers to the ratio of the intensity of the 2D peak at  $2692\text{ cm}^{-1}$  to the intensity of the G peak at  $1,580\text{ cm}^{-1}$ .

In certain embodiments, the graphenic carbon particles have a relatively low bulk density. For example, the graphenic carbon particles are characterized by having a bulk density (tap density) of less than  $0.2\text{ g/cm}^3$ , such as no more than  $0.1\text{ g/cm}^3$ . For the purposes of the present invention, the bulk density of the graphenic carbon particles is determined by placing 0.4 grams of the graphenic carbon particles in a glass measuring cylinder having a readable scale. The cylinder is raised approximately one-inch and tapped 100 times, by striking the base of the cylinder onto a hard surface, to allow the graphenic carbon particles to settle within the cylinder. The volume of the particles is then measured, and the bulk density is calculated by dividing 0.4 grams by the measured volume, wherein the bulk density is expressed in terms of  $\text{g/cm}^3$ .

In certain embodiments, the graphenic carbon particles have a compressed density and a percent densification that is less than the compressed density and percent densification of graphite powder and certain types of substantially flat graphenic carbon particles such as those formed from exfoliated graphite. Lower compressed density and lower percent densification are each currently believed to contribute to better dispersion and/or rheological properties than graphenic carbon particles exhibiting higher compressed density and higher percent densification. In certain embodiments, the compressed density of the graphenic carbon particles is 0.9 or less, such as less than 0.8, less than 0.7, such as from 0.6 to 0.7. In certain embodiments, the percent densification of the graphenic carbon particles is less than 40%, such as less than 30%, such as from 25 to 30%.

For purposes of the present invention, the compressed density of graphenic carbon particles is calculated from a measured thickness of a given mass of the particles after compression. Specifically, the measured thickness is determined by subjecting 0.1 grams of the graphenic carbon particles to cold press under 15,000 pound of force in a 1.3 centimeter die for 45 minutes, wherein the contact pressure is 500 MPa. The compressed density of the graphenic carbon particles is then calculated from this measured thickness according to the following equation:

$$\text{Compressed Density (g/cm}^3\text{)} = \frac{0.1 \text{ grams}}{\pi * (1.3 \text{ cm}/2)^2 * (\text{measured thickness in cm})}$$

The percent densification of the graphenic carbon particles is then determined as the ratio of the calculated compressed density of the graphenic carbon particles, as determined above, to  $2.2\text{ g/cm}^3$ , which is the density of graphite.

In certain embodiments, the graphenic carbon particles have a measured bulk liquid conductivity of at least 100 microSiemens, such as at least 120 microSiemens, such as at least 140 microSiemens immediately after mixing and at later points in time, such as at 10 minutes, or 20 minutes, or 30 minutes, or 40 minutes. For the purposes of the present invention, the bulk liquid conductivity of the graphenic carbon particles is determined as follows. First, a sample comprising a 0.5% solution of graphenic carbon particles in butyl cellosolve is sonicated for 30 minutes with a bath sonicator. Immediately following sonication, the sample is

placed in a standard calibrated electrolytic conductivity cell (K=1). A Fisher Scientific AB 30 conductivity meter is introduced to the sample to measure the conductivity of the sample. The conductivity is plotted over the course of about 40 minutes.

In accordance with certain embodiments, percolation, defined as long range interconnectivity, occurs between the conductive graphenic carbon particles. Such percolation may reduce the resistivity of the coating compositions. The conductive graphenic particles may occupy a minimum volume within the coating such that the particles form a continuous, or nearly continuous, network. In such a case, the aspect ratios of the graphenic carbon particles may affect the minimum volume required for percolation.

In certain embodiments, at least a portion of the graphenic carbon particles to be dispersed in the compositions of the present invention are made by thermal processes. In accordance with embodiments of the invention, thermally produced graphenic carbon particles are made from carbon-containing precursor materials that are heated to high temperatures in a thermal zone such as a plasma. As more fully described below, the carbon-containing precursor materials are heated to a sufficiently high temperature, e.g., above 3,500° C., to produce graphenic carbon particles having characteristics as described above. The carbon-containing precursor, such as a hydrocarbon provided in gaseous or liquid form, is heated in the thermal zone to produce the graphenic carbon particles in the thermal zone or downstream therefrom. For example, thermally produced graphenic carbon particles may be made by the systems and methods disclosed in U.S. Pat. Nos. 8,486,363 and 8,486,364.

In certain embodiments, the thermally produced graphenic carbon particles may be made by using the apparatus and method described in U.S. Pat. No. 8,486,363 at [0022] to [0048] in which (i) one or more hydrocarbon precursor materials capable of forming a two-carbon fragment species (such as n-propanol, ethane, ethylene, acetylene, vinyl chloride, 1,2-dichloroethane, allyl alcohol, propionaldehyde, and/or vinyl bromide) is introduced into a thermal zone (such as a plasma), and (ii) the hydrocarbon is heated in the thermal zone to form the graphenic carbon particles. In other embodiments, the thermally produced graphenic carbon particles may be made by using the apparatus and method described in U.S. Pat. No. 8,486,364 at [0015] to [0042] in which (i) a methane precursor material (such as a material comprising at least 50 percent methane, or, in some cases, gaseous or liquid methane of at least 95 or 99 percent purity or higher) is introduced into a thermal zone (such as a plasma), and (ii) the methane precursor is heated in the thermal zone to form the graphenic carbon particles. Such methods can produce graphenic carbon particles having at least some, in some cases all, of the characteristics described above.

During production of the graphenic carbon particles by the thermal production methods described above, a carbon-containing precursor is provided as a feed material that may be contacted with an inert carrier gas. The carbon-containing precursor material may be heated in a thermal zone, for example, by a plasma system. In certain embodiments, the precursor material is heated to a temperature of at least 3,500° C., for example, from a temperature of greater than 3,500° C. or 4,000° C. up to 10,000° C. or 20,000° C. Although the thermal zone may be generated by a plasma system, it is to be understood that any other suitable heating

system may be used to create the thermal zone, such as various types of furnaces including electrically heated tube furnaces and the like.

The gaseous stream may be contacted with one or more quench streams that are injected into the plasma chamber through at least one quench stream injection port. The quench stream may cool the gaseous stream to facilitate the formation or control the particle size or morphology of the graphenic carbon particles. In certain embodiments of the invention, after contacting the gaseous product stream with the quench streams, the ultrafine particles may be passed through a converging member. After the graphenic carbon particles exit the plasma system, they may be collected. Any suitable means may be used to separate the graphenic carbon particles from the gas flow, such as, for example, a bag filter, cyclone separator or deposition on a substrate.

In certain embodiments, at least a portion of the graphenic carbon particles may be obtained from commercial sources, for example, from Angstrom, XG Sciences and other commercial sources. In such embodiments, the commercially available graphenic carbon particles may comprise exfoliated graphite and have different characteristics in comparison with the thermally produced graphenic carbon particles, such as different size distributions, thicknesses, aspect ratios, structural morphologies, oxygen contents, and chemical functionalities at the basal planes/edges.

In certain embodiments, the graphenic carbon particles are functionalized. As used herein, "functionalized", when referring to graphenic carbon particles, means covalent bonding of any non-carbon atom or any organic group to the graphenic carbon particles. The graphenic carbon particles may be functionalized through the formation of covalent bonds between the carbon atoms of a particle and other chemical moieties such as carboxylic acid groups, sulfonic acid groups, hydroxyl groups, halogen atoms, nitro groups, amine groups, aliphatic hydrocarbon groups, phenyl groups and the like. For example, functionalization with carbonaceous materials may result in the formation of carboxylic acid groups on the graphenic carbon particles. The graphenic carbon particles may also be functionalized by other reactions such as Diels-Alder addition reactions, 1,3-dipolar cycloaddition reactions, free radical addition reactions and diazonium addition reactions. In certain embodiments, the hydrocarbon and phenyl groups may be further functionalized. If the graphenic carbon particles already have some hydroxyl functionality, the functionality can be modified and extended by reacting these groups with, for example, an organic isocyanate.

In certain embodiments, different types of graphenic carbon particles may be co-dispersed in the composition. For example, when thermally produced graphenic carbon particles are combined with commercially available graphenic carbon particles in accordance with embodiments of the invention, a bi-modal distribution, tri-modal distribution, etc. of graphenic carbon particle characteristics may be achieved. The graphenic carbon particles contained in the compositions may have multi-modal particle size distributions, aspect ratio distributions, structural morphologies, edge functionality differences, oxygen content, and the like.

In an embodiment of the present invention in which both thermally produced graphenic carbon particles and commercially available graphenic carbon particles, e.g., from exfoliated graphite, are co-dispersed and added to a coating composition to produce a bi-modal graphenic particle size distribution, the relative amounts of the different types of graphenic carbon particles are controlled to produce desired conductivity properties of the coatings. For example, the

thermally produced graphenic particles may comprise from 1 to 50 weight percent, and the commercially available graphenic carbon particles may comprise from 50 to 99 weight percent, based on the total weight of the graphenic carbon particles. In certain embodiments, the thermally produced graphenic carbon particles may comprise from 2 or 4 to 40 weight percent, or from 6 or 8 to 35 weight percent, or from 10 to 30 weight percent. When co-dispersions of the present invention having such relative amounts of thermally produced graphenic carbon particles and commercially available graphenic carbon particles are incorporated in coatings, inks, or other materials, such materials may exhibit significantly increased electrical conductivities in comparison with similar materials containing mixtures of such types of graphenic carbon particles at similar ratios. For example, the co-dispersions may increase electrical conductivity by at least 10 or 20 percent compared with the mixtures. In certain embodiments, the electrical conductivity may be increased by at least 50, 70 or 90 percent, or more.

In certain embodiments, the coating compositions or other materials produced with the present dispersions are substantially free of certain components such as polyalkyleneimines, graphite, or other components. For example, the term "substantially free of polyalkyleneimines" means that polyalkyleneimines are not purposefully added, or are present as impurities or in trace amounts, e.g., less than 1 weight percent or less than 0.1 weight percent. The term "substantially free of graphite" means that graphite is not purposefully added, or is present as an impurity or in trace amounts, e.g., less than 1 weight percent or less than 0.1 weight percent. In certain embodiments, graphite in minor amounts may be present in the materials, e.g., less than 5 weight percent or less than 1 weight percent of the material. If graphite is present, it is typically in an amount less than the graphenic carbon particles, e.g., less than 30 weight percent based on the combined weight of the graphite and graphenic carbon particles, for example, less than 20 or 10 weight percent.

In certain embodiments, the compositions of the present invention are prepared from a dispersion comprising: (a) graphenic carbon particles such as any of those described above; (b) a carrier that may be selected from water, at least one organic solvent, or combinations of water and at least one organic solvent; (c) at least one polymeric dispersant, such as the copolymer described generally below; and, optionally, (d) at least one resin as described above or other additives.

Certain compositions of the present invention comprise at least one polymeric dispersant. In certain embodiments, such a polymeric dispersant comprises a tri-block copolymer comprising: (i) a first segment comprising graphenic carbon affinic groups, such as hydrophobic aromatic groups; (ii) a second segment comprising polar groups, such as hydroxyl groups, amine groups, ether groups, and/or acid groups; and (iii) a third segment which is different from the first segment and the second segment, such as a segment that is substantially non-polar, i.e., substantially free of polar groups. As used herein, term "substantially free" when used with reference to the absence of groups in a polymeric segment, means that no more than 5% by weight of the monomer used to form the third segment comprises polar groups.

Suitable polymeric dispersants include acrylic copolymers produced from atom transfer radical polymerization. In certain embodiments, such copolymers have a weight average molecular weight of 1,000 to 20,000.

In certain embodiments, the polymeric pigment dispersant has a polymer chain structure represented by the following general formula (I),



wherein G is a residue of at least one radically polymerizable ethylenically unsaturated monomer; W and Y are residues of at least one radically polymerizable ethylenically unsaturated monomer with W and Y being different from one another; Y is optional;  $\Phi$  is a hydrophobic residue of or derived from an initiator and is free of the radically transferable group; T is or is derived from the radically transferable group of the initiator; p, q and s represent average numbers of residues occurring in a block of residues; p, q and s are each individually selected such that the polymeric dispersant has a number average molecular weight of at least 250.

The polymeric dispersant may be described generally as having a head and tail structure, i.e., as having a polymeric head portion and a polymeric tail portion. The polymeric tail portion may have a hydrophilic portion and a hydrophobic portion, particularly at the terminus thereof. While not intending to be bound by any theory, it is believed that the polymeric head portion of the polymeric dispersant can be associated with the graphenic carbon particles, while the polymeric tail portion aids in dispersing the graphenic carbon particles and can be associated with other components of an ink or coating composition. As used herein, the terms "hydrophobic" and "hydrophilic" are relative to each other.

In certain embodiments, the polymeric dispersant is prepared by atom transfer radical polymerization (ATRP). The ATRP process can be described generally as comprising: polymerizing one or more radically polymerizable monomers in the presence of an initiation system; forming a polymer; and isolating the formed polymer. In certain embodiments, the initiation system comprises: a monomeric initiator having a single radically transferable atom or group; a transition metal compound, i.e., a catalyst, which participates in a reversible redox cycle with the initiator; and a ligand, which coordinates with the transition metal compound. The ATRP process is described in further detail in International Patent Publication No. WO 98/40415 and U.S. Pat. Nos. 5,807,937, 5,763,548 and 5,789,487.

Catalysts that may be used in the ATRP preparation of the polymeric dispersant include any transition metal compound that can participate in a redox cycle with the initiator and the growing polymer chain. It may be preferred that the transition metal compound not form direct carbon-metal bonds with the polymer chain. Transition metal catalysts useful in the present invention may be represented by the following general formula (II),



wherein M is the transition metal; n is the formal charge on the transition metal having a value of from 0 to 7; and X is a counterion or covalently bonded component. Examples of the transition metal M include, but are not limited to, Cu, Fe, Au, Ag, Hg, Pd, Pt, Co, Mn, Ru, Mo, Nb and Zn. Examples of X include, but are not limited to, halide, hydroxy, oxygen,  $C_1-C_6$ -alkoxy, cyano, cyanato, thiocyanato and azido. In one specific example, the transition metal is Cu(I) and X is halide, for example, chloride. Accordingly, one specific class of transition metal catalysts is the copper halides, for example, Cu(I)Cl. In certain embodiments, the transition metal catalyst may contain a small amount, for example, 1 mole percent, of a redox conjugate, for example, Cu(II)Cl<sub>2</sub>

## 11

when Cu(I)Cl is used. Additional catalysts useful in preparing the polymeric dispersant are described in U.S. Pat. No. 5,807,937 at column 18, lines 29 through 56. Redox conjugates are described in further detail in U.S. Pat. No. 5,807,937 at column 11, line 1 through column 13, line 38.

Ligands that may be used in the ATRP preparation of the polymeric dispersant include, but are not limited to, compounds having one or more nitrogen, oxygen, phosphorus and/or sulfur atoms, which can coordinate to the transition metal catalyst compound, for example, through sigma and/or pi bonds. Classes of useful ligands include, but are not limited to, unsubstituted and substituted pyridines and bipyridines; porphyrins; cryptands; crown ethers; for example, 18-crown-6; polyamines, for example, ethylenediamine; glycols, for example, alkylene glycols, such as ethylene glycol; carbon monoxide; and coordinating monomers, for example, styrene, acrylonitrile and hydroxyalkyl (meth)acrylates. As used herein, the term "(meth)acrylate" and similar terms refer to acrylates, methacrylates and mixtures of acrylates and methacrylates. One specific class of ligands are the substituted bipyridines, for example, 4,4'-dialkyl-bipyridyls. Additional ligands that may be used in preparing polymeric dispersant are described in U.S. Pat. No. 5,807,937 at column 18, line 57 through column 21, line 43.

Classes of monomeric initiators that may be used in the ATRP preparation of the polymeric dispersant include, but are not limited to, aliphatic compounds, cycloaliphatic compounds, aromatic compounds, polycyclic aromatic compounds, heterocyclic compounds, sulfonyl compounds, sulphenyl compounds, esters of carboxylic acids, nitrites, ketones, phosphonates and mixtures thereof, each having a radically transferable group, and preferably a single radically transferable group. The radically transferable group of the monomeric initiator may be selected from, for example, cyano, cyanato, thiocyanato, azido and halide groups. The monomeric initiator may also be substituted with functional groups, for example, oxyranyl groups, such as glycidyl groups. Additional useful initiators are described in U.S. Pat. No. 5,807,937 at column 17, line 4 through column 18, line 28.

In certain embodiments, the monomeric initiator is selected from 1-halo-2,3-epoxypropane, p-toluenesulfonyl halide, p-toluenesulphenyl halide, C<sub>6</sub>-C<sub>20</sub>-alkyl ester of alpha-halo-C<sub>2</sub>-C<sub>6</sub>-carboxylic acid, halomethylbenzene, (1-haloethyl)benzene, halomethylnaphthalene, halomethylanthracene and mixtures thereof. Examples of C<sub>2</sub>-C<sub>6</sub>-alkyl ester of alpha-halo-C<sub>2</sub>-C<sub>6</sub>-carboxylic acids include, hexyl alpha-bromopropionate, 2-ethylhexyl alpha-bromopropionate, 2-ethylhexyl alpha-bromohexionate and icosanyl alpha-bromo-propionate. As used herein, the term "monomeric initiator" is meant to be distinguishable from polymeric initiators, such as polyethers, polyurethanes, polyesters and acrylic polymers having radically transferable groups.

In the ATRP preparation, the polymeric dispersant and the amounts and relative proportions of monomeric initiator, transition metal compound and ligand may be those for which ATRP is most effectively performed. The amount of initiator used can vary widely and is typically present in the reaction medium in a concentration of from 10<sup>-4</sup> moles/liter (M) to 3 M, for example, from 10<sup>-3</sup> M to 10<sup>-1</sup> M. As the molecular weight of the polymeric dispersant can be directly related to the relative concentrations of initiator and monomer(s), the molar ratio of initiator to monomer is an important factor in polymer preparation. The molar ratio of initiator to monomer is typically within the range of 10<sup>-4</sup>:1 to 0.5:1, for example, 10<sup>-3</sup>:1 to 5×10<sup>-2</sup>:1.

## 12

In preparing the polymeric dispersant by ATRP methods, the molar ratio of transition metal compound to initiator is typically in the range of 10<sup>-4</sup>:1 to 10:1, for example, 0.1:1 to 5:1. The molar ratio of ligand to transition metal compound is typically within the range of 0.1:1 to 100:1, for example, 0.2:1 to 10:1.

The polymeric dispersant may be prepared in the absence of solvent, i.e., by means of a bulk polymerization process. Often, the polymeric dispersant is prepared in the presence of a solvent, typically water and/or an organic solvent. Classes of useful organic solvents include, but are not limited to, esters of carboxylic acids, ethers, cyclic ethers, C<sub>5</sub>-C<sub>10</sub> alkanes, C<sub>5</sub>-C<sub>8</sub> cycloalkanes, aromatic hydrocarbon solvents, halogenated hydrocarbon solvents, amides, nitrates, sulfoxides, sulfones and mixtures thereof. Super-critical solvents, such as CO<sub>2</sub>, C<sub>1</sub>-C<sub>4</sub> alkanes and fluorocarbons, may also be employed. One class of solvents is the aromatic hydrocarbon solvents, such as xylene, toluene, and mixed aromatic solvents such as those commercially available from Exxon Chemical America under the trademark SOLVESSO. Additional solvents are described in further detail in U.S. Pat. No. 5,807,937, at column 21, line 44 through column 22, line 54.

The ATRP preparation of the polymeric dispersant is typically conducted at a reaction temperature within the range of 25° C. to 140° C., for example, from 50° C. to 100° C., and a pressure within the range of 1 to 100 atmospheres, usually at ambient pressure.

The ATRP transition metal catalyst and its associated ligand are typically separated or removed from the polymeric dispersant prior to its use in the polymeric dispersants of the present invention. Removal of the ATRP catalyst may be achieved using known methods, including, for example, adding a catalyst binding agent to the mixture of the polymeric dispersant, solvent and catalyst, followed by filtering. Examples of suitable catalyst binding agents include, for example, alumina, silica, clay or a combination thereof. A mixture of the polymeric dispersant, solvent and ATRP catalyst may be passed through a bed of catalyst binding agent. Alternatively, the ATRP catalyst may be oxidized in situ, the oxidized residue of the catalyst being retained in the polymeric dispersant.

With reference to general formula (I), G may be a residue of at least one radically polymerizable ethylenically unsaturated monomer, such as a monomer selected from an oxirane functional monomer reacted with a carboxylic acid which may be an aromatic carboxylic acid or polycyclic aromatic carboxylic acid.

The oxirane functional monomer or its residue that is reacted with a carboxylic acid may be selected from, for example, glycidyl (meth)acrylate, 3,4-epoxycyclohexylmethylethyl(meth)acrylate, 2-(3,4-epoxycyclohexyl)ethyl(meth)acrylate, allyl glycidyl ether and mixtures thereof. Examples of carboxylic acids that may be reacted with the oxirane functional monomer or its residue include, but are not limited to, naphthoic acid, hydroxy naphthoic acids, para-nitrobenzoic acid and mixtures thereof.

With continued reference to general formula (I), in certain embodiments, W and Y may each independently be residues of, include, but are not limited to, methyl (meth)acrylate, ethyl (meth)acrylate, propyl (meth)acrylate, isopropyl (meth)acrylate, n-butyl (meth)acrylate, iso-butyl (meth)acrylate, tert-butyl (meth)acrylate, 2-ethylhexyl (meth)acrylate, lauryl (meth)acrylate, isobornyl (meth)acrylate, cyclohexyl (meth)acrylate, 3,3,5-trimethylcyclohexyl (meth)acrylate, isocane (meth)acrylate, hydroxyethyl (meth)acrylate, hydroxypropyl (meth)acrylate, hydroxybutyl

(meth)acrylate, butyl (meth)acrylate, methoxy poly(ethylene glycol)mono(meth)acrylate, poly(ethylene glycol)mono (meth)acrylate, methoxy poly(propylene glycol)mono (meth)acrylate, poly(propylene glycol)mono(meth)acrylate, methoxy copoly(ethylene glycol/propylene glycol)mono (meth)acrylate, copoly(ethylene glycol/propylene glycol)mono(meth)acrylate.

In general formula (I), in certain embodiments, W and Y may each independently be residues of monomers having more than one (meth)acryloyl group, such as (meth)acrylic anhydride, diethyleneglycol bis(meth)acrylate, 1,4-butanediol diacrylate, 1,6-hexanediol diacrylate, 4,4'-isopropylidenediphenol bis(meth)acrylate (Bisphenol A di(meth)acrylate), alkoxylated 4,4'-isopropylidenediphenol bis (meth)acrylate, trimethylolpropane tris(meth)acrylate, alkoxylated trimethylolpropane tris(meth)acrylate, polyethylene glycol di(meth)acrylate, polypropylene glycol di(meth)acrylate, and copoly(ethylene glycol/propylene glycol)di(meth)acrylate.

The numerals p, q and s represent the average total number of G, W and Y residues, respectively, occurring per block or segment of G residues (G-block or G-segment), W residues (W-block or W-segment) and Y residues (Y-block G or Y-segment), respectively. When containing more than one type or species of monomer residue, the W- and Y-blocks may each have at least one of random block (e.g., di-block and tri-block), alternating, and gradient architectures. Gradient architecture refers to a sequence of different monomer residues that change gradually in a systematic and predictable manner along the polymer backbone. For purposes of illustration, a W-block containing 6 residues of butyl methacrylate (B MA) and 6 residues of hydroxy propyl methacrylate (HPMA), for which q is 12, may have di-block, tetra-block, alternating and gradient architectures as described in U.S. Pat. No. 6,642,301, col. 10, lines 5-25. In certain embodiments, the G-block may include about 5-15 residues of glycidyl(meth)acrylate reacted with an aromatic carboxylic acid (such as 3-hydroxy-2-napthoic acid), the W-block may be a random block of about 20-30 BMA and HPMA residues and the Y-block may be a uniform block of about 5-15 butyl acrylate (BA) residues.

The order in which monomer residues occur along the polymer backbone of the polymeric dispersant is typically determined by the order in which the corresponding monomers are fed into the vessel in which the controlled radical polymerization is conducted. For example, the monomers that are incorporated as residues in the G-block of the polymeric dispersant are generally fed into the reaction vessel prior to those monomers that are incorporated as residues in the W-block, followed by the residues of the Y-block.

During formation of the W- and Y-blocks, if more than one monomer is fed into the reaction vessel at a time, the relative reactivities of the monomers typically determines the order in which they are incorporated into the living polymer chain. Gradient sequences of monomer residues within the W- and Y-blocks can be prepared by controlled radical polymerization, and, in particular, by ATRP methods by (a) varying the ratio of monomers fed to the reaction medium during the course of the polymerization, (b) using a monomer feed containing monomers having different rates of polymerization, or (c) a combination of (a) and (b). Copolymers containing gradient architecture are described in further detail in U.S. Pat. No. 5,807,937, at column 29, line 29 through column 31, line 35.

In certain embodiments, subscripts q and s each have a value of at least 1, such as at least 5 for general formula (I).

Also, subscript s often has a value of less than 300, such as less than 100, or less than 50 (for example 20 or less) for general formula (I). The values of subscripts q and s may range between any combination of these values, inclusive of the recited values, for example, s may be a number from 1 to 100. Subscript p may have a value of at least 1, such as at least 5. Subscript p also often has a value of less than 300, such as less than 100 or less than 50 (e.g., 20 or less). The value of subscript p may range between any combination of these values, inclusive of the recited values, for example, p may be a number up to 50. The polymeric dispersant often has a number average molecular weight (Mn) of from 250 to 40,000, for example, from 1000 to 30,000 or from 2000 to 20,000, as determined by gel permeation chromatography using polystyrene standards.

Symbol  $\Phi$  of general formula (I) is, or is derived from, the residue of the initiator used in the preparation of the polymeric dispersant by controlled radical polymerization, and is free of the radically transferable group of the initiator. For example, when the polymeric dispersant is initiated in the presence of toluene sulfonyl chloride, the symbol  $\Phi$ , more specifically  $\Phi^-$  is the residue,



The symbol  $\Phi$  may also represent a derivative of the residue of the initiator.

In general formula (I), T is or is derived from the radically transferable group of the ATRP initiator. The residue of the radically transferable group may be (a) left on the polymeric dispersant, (b) removed or (c) chemically converted to another moiety. The radically transferable group may be removed by substitution with a nucleophilic compound, for example, an alkali metal alkoxylate. When the residue of the radically transferable group is, for example, a cyano group (—CN), it can be converted to an amide group or carboxylic acid group by methods known in the art.

The polymeric dispersant is typically present in the graphenic carbon particle dispersion described above in an amount of at least 0.1 percent by weight, such as at least 0.5 percent by weight, or, in some cases, at least 1 percent by weight, based on the total weight of the graphenic carbon particle dispersion. The polymeric dispersant may typically be present in the graphenic carbon particle dispersion in an amount of less than 75 percent by weight, or less than 50 percent by weight, based on the total weight of the graphenic carbon particle dispersion. In certain embodiments, the polymeric dispersant may be present in the graphenic carbon particle dispersion in an amount of less than 30 percent by weight, or less than 15 percent by weight, based on the total weight of the graphenic carbon particle dispersion.

The graphenic carbon particle dispersion often also comprises at least water and/or at least one organic solvent. Classes of organic solvents that may be present include, but are not limited to, xylene, toluene, alcohols, for example, methanol, ethanol, n-propanol, iso-propanol, n-butanol, sec-butyl alcohol, tert-butyl alcohol, iso-butyl alcohol, furfuryl alcohol and tetrahydrofurfuryl alcohol; ketones or ketoalco-

## 15

hols, for example, acetone, methyl ethyl ketone, and diacetone alcohol; ethers, for example, dimethyl ether and methyl ethyl ether; cyclic ethers, for example, tetrahydro-

## 16

n-methyl-2-pyrrolidone before filtering off the milling media. The P/B (pigment to binder ratio) in each composition is 6.

TABLE 1

|        | Dispersions |      |     |     |     |     |     |     |     |     |
|--------|-------------|------|-----|-----|-----|-----|-----|-----|-----|-----|
|        | Sample:     |      |     |     |     |     |     |     |     |     |
|        | A           | B    | C   | D   | E   | F   | G   | H   | I   | J   |
| % M-25 | 0           | 100  | 100 | 90  | 85  | 80  | 75  | 70  | 60  | 50  |
| % TGC  | 100         | 0    | 0   | 10  | 15  | 20  | 25  | 30  | 40  | 50  |
| % TS   | 6.0         | 10.7 | 8.6 | 8.7 | 8.3 | 8.2 | 8.2 | 7.5 | 9.5 | 9.1 |

furan and dioxane; esters, for example, ethyl acetate, ethyl lactate, ethylene carbonate and propylene carbonate; polyhydric alcohols, for example, ethylene glycol, diethylene glycol, triethylene glycol, propylene glycol, tetraethylene glycol, polyethylene glycol, glycerol, 2-methyl-2,4-pentanediol and 1,2,6-hexanetriol; hydroxy functional ethers of alkylene glycols, for example, butyl 2-hydroxyethyl ether, hexyl 2-hydroxyethyl ether, methyl 2-hydroxypropyl ether and phenyl 2-hydroxypropyl ether; nitrogen containing cyclic compounds, for example, pyrrolidone, N-methyl-2-pyrrolidone and 1,3-dimethyl-2-imidazolidinone; and sulfur containing compounds such as thioglycol, dimethyl sulfoxide and tetramethylene sulfone. When the solvent comprises water, it can be used alone or in combination with organic solvents such as propylene glycol monomethyl ether, ethanol and the like.

The graphenic carbon particle dispersion may be prepared by the use of conventional mixing techniques such as energy intensive mixing or grinding means, such as ball mills or media mills (e.g., sand mills), attritor mills, 3-roll mills, rotor/stator mixers, high speed mixers, sonicators, and the like.

The graphenic carbon particles may be mixed with film-forming resins and other components of the compositions. For example, for two-part coating systems, the graphenic carbon particles may be dispersed into part A and/or part B. In certain embodiments, the graphenic carbon particles are dispersed into part A by various mixing techniques such as sonication, high speed mixing, media milling and the like. In certain embodiments, the graphenic carbon particles may be mixed into the coating compositions using high-energy and/or high-shear techniques such as sonication, 3-roll milling, ball milling, attritor milling, rotor/stator mixers, and the like.

The following examples are intended to illustrate various aspects of the invention, and are not intended to limit the scope of the invention.

## EXAMPLE 1

The compositions summarized in Table 1 were dispersed by adding 70 g of the following composition into 8 oz. glass jars with 220 g of SEPR Ermil 1.0-1.25 mm milling media. All of the compositions were formulated comprising 60.95 g of n-methyl-2-pyrrolidone, 7.0 g total of graphenic carbon particles, and 2.05 g of solvent-born block copolymer dispersant (which comprises 43 weight % n-butyl acetate and 57 weight % block copolymer as disclosed in US 2008/0188610). The samples in the jars were shaken for 4 hours using a Lau disperser (Model DAS 200, Lau, GmbH). After shaking, the dispersions were diluted with additional

15 In Table 1, the designation M-25 stands for xGnP-M-25 exfoliated graphenic carbon particles commercially available from XG Sciences. The designation TGC stands for thermally produced graphenic carbon particles produced in accordance with the method disclosed in U.S. Pat. No. 8,486,364 having a measured BET surface area of 280 m<sup>2</sup>/g. The % TS (% total solids) of each dispersion after dilution and filtering off the milling media is shown. Sample A contains only the TGC graphenic carbon particles, while Samples B and C contain only the M-25 graphenic carbon particles. Samples D, E, F, G, H, I and J contain both types of graphenic carbon particles co-dispersed together. The weight % of each type of graphenic carbon particle relative to the total graphenic carbon particle content in each composition is shown.

## EXAMPLE 2

Sample A from Table 1 containing only TGC graphenic carbon particles was mixed with Sample B from Table 1 containing only M-25 graphenic carbon particles in different ratios, as listed below in Table 2. Each mixture was made by adding the appropriate amount of each sample together into a glass jar and vigorously stirring with a stir blade until thoroughly mixed. The P/B for each resulting composition is 6.

TABLE 2

|        | Mixtures |    |    |    |    |    |    |    |    |    |    |    |    |
|--------|----------|----|----|----|----|----|----|----|----|----|----|----|----|
|        | Sample:  |    |    |    |    |    |    |    |    |    |    |    |    |
|        | 1        | 2  | 3  | 4  | 5  | 6  | 7  | 8  | 9  | 10 | 11 | 12 | 13 |
| % M-25 | 98       | 96 | 94 | 92 | 90 | 88 | 86 | 84 | 82 | 80 | 70 | 60 | 50 |
| % TGC  | 2        | 4  | 6  | 8  | 10 | 12 | 14 | 16 | 18 | 20 | 30 | 40 | 50 |

## EXAMPLE 3

55 Samples C through J from Table 1 and Samples 1 through 13 from Table 2 were applied as 1-2 mm wide lines in a serpentine circuit pattern to a 2x3 inch glass slide (Fisherbrand, Plain, Precleaned) using a dispensing jet (PICO valve, MV-100, Nordson, EFD) and a desktop robot (2504N, Janome) and then dried in an oven at 212° F. for 30 minutes. The electrical conductivity was determined by first measuring the resistance of the serpentine circuit vs. the length of the circuit line. Then, the cross-sectional area of the serpentine lines was measured using a stylus profilometer (Dektak). Using the measured values for the cross sectional area (A) and the resistance (R) for a given length (L) of the

circuit, the resistivity ( $\rho$ ) was calculated using the equation  $\rho=RA/L$ . Then the conductivity ( $\sigma$ ) was calculated by taking the reciprocal of the resistivity,  $\sigma=1/\rho$ . Conductivity results are shown in Table 3 in units of Siemen per meter.

TABLE 3

| Electrical Conductivity |       |        |        |        |        |        |        |        |        |        |        |
|-------------------------|-------|--------|--------|--------|--------|--------|--------|--------|--------|--------|--------|
| Sample                  |       |        |        |        |        |        |        |        |        |        |        |
| C                       | 1     | 2      | 3      | 4      | 5      | 6      | 7      | 8      | 9      | 10     |        |
| % TGC                   | 0     | 2      | 4      | 6      | 8      | 10     | 12     | 14     | 16     | 18     | 20     |
| Type                    | M-25  | M      | M      | M      | M      | M      | M      | M      | M      | M      | M      |
| $\sigma$ (S/m)          | 9,502 | 11,325 | 12,151 | 12,853 | 13,038 | 14,025 | 12,500 | 12,422 | 12,903 | 11,919 | 12,771 |

  

| Sample         |        |       |       |        |        |        |        |        |       |       |  |
|----------------|--------|-------|-------|--------|--------|--------|--------|--------|-------|-------|--|
| 11             | 12     | 13    | D     | E      | F      | G      | H      | I      | J     |       |  |
| % TGC          | 30     | 40    | 50    | 10     | 15     | 20     | 25     | 30     | 40    | 50    |  |
| Type           | M      | M     | M     | C      | C      | C      | C      | C      | C     | C     |  |
| $\sigma$ (S/m) | 10,753 | 8,264 | 6,135 | 19,455 | 21,552 | 22,422 | 25,189 | 20,534 | 8,889 | 6,219 |  |

In Table 3, % TGC designates the weight % of thermally produced graphenic carbon particles of the total graphenic carbon particle content of the composition. M-25 designates the dispersion of just xGnP-M-25 (from Sample C). M designates the mixture of dispersions with two different graphenic carbon particle types (Samples 1 through 13). C designates the co-dispersions of two types of graphenic carbon particles (Samples D through J). The conductivity results listed in Table 3 are shown graphically in FIG. 1, which plots electrical conductivity versus % TGC for both the co-dispersions and the mixtures of the graphenic carbon particles.

## EXAMPLE 4

A co-dispersion is made by adding 70 g of the following composition into an 8 oz. glass jar with 350 g of Zirconox 1.0-1.2 mm media: 87.02 weight % n-methyl-2-pyrrolidone, 1.00 weight % n-butyl acetate, 7.70 weight % xGnP-M-25 exfoliated graphenic carbon particles, 2.57 weight % thermally-produced graphenic carbon particles produced in accordance with the method disclosed in U.S. Pat. No. 8,486,364 having a measured BET surface area of 280 m<sup>2</sup>/g, and 1.71 weight % of dispersant solids, where the dispersant solids arise from a 50/50 mixture of two types of solvent-born block copolymer dispersants (both of which are block copolymers as disclosed in US 2008/0188610), in which the chemical composition of the dispersants is similar, but the molecular weight of the two dispersants is different; specifically, one has a molecular weight of 9,700 g/mol, and the other has a molecular weight of 4,850 g/mol. The jar and milling media were shaken for 4 hours using a Lau disperser (Model DAS 200, Lau, GmbH). After shaking, the co-dispersion was diluted with additional n-methyl-2-pyrrolidone before filtering off the milling media. The P/B (pigment to binder ratio) of this composition is 6. The conductivity of this composition was measured to be 27,893 S/m.

## EXAMPLE 5

The compositions summarized in Table 4 were dispersed by adding 21.88 g of the following composition into 2.5 oz. glass jars with 109 g of milling media (Zirconox 1.0-1.2

mm). All of the compositions were formulated comprising 19.34 g of n-methyl-2-pyrrolidone, 2.19 g total of carbon particles, and 0.18 g of a solvent-born block copolymer dispersant comprising 39.89 weight % n-butyl acetate and

60.11 weight % block copolymer as disclosed in US2008/0188610 with a molecular weight of 9,700 g/mol, and 0.17 g of a solvent-born block copolymer dispersant comprising 33.73 weight % n-butyl acetate and 66.27 weight % block copolymer as disclosed in US 2008/0188610 with a molecular weight of 4,850 g/mol. The samples in the jars were shaken for 4 hours using a Lau disperser (Model DAS 200, Lau, GmbH). Extra n-methyl-2-pyrrolidone (from 0 g up to 6.25 g) was added after milling to enable easier filtration of the product from the milling media. The milling media were then filtered off from the dispersions. The final % total solids were then measured. The P/B (pigment to binder ratio) in each composition is 10.

Each of these compositions (Samples K, L and M) were applied as 1-2 mm wide lines in a serpentine circuit pattern to a 2x3 inch glass slide (Fisherbrand, Plain, Precleaned) using a dispensing jet (PICO valve, MV-100, Nordson, EFD) and a desktop robot (2504N, Janome) and then dried in an oven at 212° F. for 30 minutes. The electrical conductivity for each composition was determined by first measuring the resistance of the dried circuit lines vs. the length of the circuit lines using a digital multi-meter (DVM890, Velleman). Then, the cross-sectional areas of the circuit lines were measured using a stylus profilometer (Dektak). For each composition, using the measured values for the cross sectional area (A) and the resistance (R) for a given length (L) of the circuit lines, the resistivity ( $\rho$ ) was calculated using the equation  $\rho=RA/L$ . Then the conductivity ( $\sigma$ ) was calculated by taking the reciprocal of the resistivity,  $\sigma=1/\rho$ .

TABLE 4

| Dispersions           |        |        |      |
|-----------------------|--------|--------|------|
| Sample                |        |        |      |
|                       | K      | L      | M    |
| % Functionalized M-25 | 75     | 100    | 0    |
| % TGC                 | 25     | 0      | 0    |
| % Graphite            | 0      | 0      | 100  |
| % TS                  | 8.3    | 11.2   | 10.8 |
| $\sigma$ (S/m)        | 55,377 | 34,935 | 515  |

In Table 4, the designation Functionalized M-25 stands for xGnP-M-25 exfoliated graphenic carbon particles com-

19

mercially available from XG Sciences, which has been functionalized by refluxing 10 g of M25 in 500 ml of nitric acid (ACS Reagent, 70%) at 120° C. for 2 hrs, filtering and washing well with distilled water. The oxygen content is increased from less than 1% to greater than 4% by this process as measured by XPS. The designation TGC stands for thermally produced graphenic carbon particles produced in accordance with the method disclosed in U.S. Pat. No. 8,486,364 having a measured BET surface area of 280 m<sup>2</sup>/g. The Graphite is C-nergy SFG6 L Graphite AL-010, from Timcal. The % TS (% total solids) of each dispersion after dilution and filtering off the milling media is shown. Sample K contains both types of graphenic carbon particles (M25 and TGC) co-dispersed together. Sample L contains only functionalized M25 graphenic carbon particles. Sample M contains no graphenic carbon particles, and contains a single type of carbon particle, namely, graphite.

## EXAMPLE 6

Sample C was applied onto a cleaned glass panel (4x8 inches) using a multiple clearance square applicator (2 inch square frame, Cat. No. 5361, from Byk Additives & Instruments) at 1 mil wet film thickness. The panel with the applied coating was baked in an oven for 30 minutes at 212° F. Wire Glue<sup>TM</sup> (conductive glue from Idolon Technologies) was used to glue copper wire electrodes at the ends of the coating to thereby produce a test panel similar to that shown in FIG. 2. The glue dried for 24 hours. The thickness of the coating was measured with an optical profilometer (Veeco Wyko NT3300 run in VSI mode) to be 2.2 μm. The resistance between the electrodes was measured to be 183 ohms using a digital multi-meter (DVM890, Velleman). In a resistive heating experiment, an electrical potential of 60 V was applied to the copper wire electrodes using a Xantrex HPD 60-5 power supply, and the temperature of the glass plate was then measured between the electrodes using a Fluke 62 Max IR thermometer. The temperature at the center of the glass plate rose from 73° F. to 138° F. in 12.3 minutes, as graphically shown in FIG. 3.

## EXAMPLE 7

Sample G was diluted with n-methyl-2-pyrrolidone to a total solids value of 5.2%. The diluted sample was then applied onto a cleaned glass panel (4x8 inches) using a multiple clearance square applicator (2 inch square frame, Cat. No. 5361, from Byk Additives & Instruments) at 2 mil wet film thickness. The panel with the applied coating was baked in an oven for 30 minutes at 212° F. Wire Glue<sup>TM</sup> (conductive glue from Idolon Technologies) was used to glue copper wire electrodes at the ends of the coating to thereby produce a test panel similar to that shown in FIG. 2. The glue dried for 24 hours. The resistance between the electrodes was measured to be 54.3 ohms using a digital multi-meter (DVM890, Velleman). In a resistive heating experiment, an electrical potential of 60 V was applied to the copper wire electrodes using a Xantrex HPD 60-5 power supply, and the temperature of the glass plate was then measured between the electrodes using a Fluke 62 Max IR thermometer. The temperature at the center of the glass plate rose from 78° F. to 230° F. in 2.2 minutes, as graphically shown in FIG. 3.

## EXAMPLE 8

Sample K, L and M were applied onto 4x12 inch, primed, metal panels (ACT Test Panels, 04X12X032, Item No.

20

54476, C710059, ED6060C, HP78) using a multiple clearance square applicator (2 inch square frame, Cat. No. 5361, from Byk Additives & Instruments) at 8 mil wet film thickness. The panels with the applied coatings dried for 3 days and were then baked in an oven for 30 minutes at 212° F. Wire Glue<sup>TM</sup> (conductive glue from Idolon Technologies) was used to glue copper wire electrodes at the ends of the coating to thereby produce test panels similar to that shown in FIG. 4. The glue dried for 24 hours. Table 5 shows dry film thickness (DFT) measurements, resistance measurements, and the results of resistive heating experiments with these panels. The thickness of the coating on each panels was measured with an optical profilometer (Veeco Wyko NT3300 run in VSI mode). The resistance between the electrodes was measured using a digital multi-meter (DVM890, Velleman). In the resistive heating experiments, an electrical potential of only 6 V was applied to the copper wire electrodes using a Hewlett Packard E3610A DC power supply, and the temperature of the metal panel between the electrodes was then measured using a Fluke 62 Max IR thermometer. The temperature is plotted vs. time in FIG. 5.

TABLE 5

|                                 | Resistive Heating Panels |      |      |
|---------------------------------|--------------------------|------|------|
|                                 | Panel made from Sample   |      |      |
|                                 | K                        | L    | M    |
| DFT (μm)                        | 13.6                     | 12.2 | 5.6  |
| Resistance (ohms)               | 3.6                      | 9.5  | 19.4 |
| Applied voltage (V)             | 6.01                     | 6.01 | 6.01 |
| Current (A)                     | 1.76                     | 0.65 | 0.31 |
| Power (W)                       | 10.58                    | 3.91 | 1.86 |
| Temperature rise in 60 s (° C.) | 27.9                     | 9.9  | 7.0  |

Table 5 and FIG. 5 show the advantage of the graphenic carbon particle coatings (panels with Samples K and L) compared to the graphite coatings (panel with Sample M). In particular, the panel with Sample K shows exceptional heating (27.9° F. temperature increase) with only 6 V of applied voltage and from only a 13.6 μm thick film.

## EXAMPLE 9

A co-dispersion was made by adding into a 2.5 oz. jar, 109 g of Zirconox 1.0-1.2 mm milling media, and the following ingredients: 0.18 g of a solvent-born block copolymer dispersant comprising 39.89 weight % n-butyl acetate and 60.11 weight % block copolymer as disclosed in US 2008/0188610 with a molecular weight of 9700 g/mol, and 0.17 g of a solvent-born block copolymer dispersant comprising 33.73 weight % n-butyl acetate and 66.27 weight % block copolymer as disclosed in US 2008/0188610 with a molecular weight of 4850 g/mol, 19.34 g of n-methyl-2-pyrrolidone, 1.64 g of xGnP-M-25 exfoliated graphenic carbon particles commercially available from XG Sciences, which had been functionalized by refluxing 10 g of the exfoliated graphenic carbon particles in 500 ml of nitric acid (ACS Reagent, 70%) at 120° C. for 2 hrs, and filtering and washing well with distilled water, and 0.55 g of thermally produced graphenic carbon particles produced in accordance with the method disclosed in U.S. Pat. No. 8,486,364 having a measured BET surface area of 280 m<sup>2</sup>/g, and which had been functionalized by adding 25 g of the thermally produced graphenic carbon particles to 3.75 g of sulfanilic acid

21

in 225 g of DI water at 80° C. with stirring, then adding gradually 1.50 g of sodium nitrite in 6 g of DI water and rinsing it in with a further 6 g of water. The reaction was cooled after gas evolution ceased and the graphenic carbon particles were filtered, washed with 10% sulfuric acid and then with water before drying at 80° C. for 2 hrs. The jar was shaken for 4 hours using a Lau disperser (Model DAS 200, Lau, GmbH). After shaking, the co-dispersion was diluted with additional n-methyl-2-pyrrolidone before filtering off the milling media. The P/B (pigment to binder ratio) of this composition was 10. The final weight % of total solids was 8.75%. This sample was applied as 1-2 mm wide lines in a serpentine circuit pattern to a 2x3 inch glass slide (Fisherbrand, Plain, Precleaned) using a dispensing jet (PICO valve, MV-100, Nordson, EFD) and a desktop robot (2504N, Janome) and then dried in an oven at 212° F. for 30 minutes. The electrical conductivity the sample was determined by first measuring the resistance of the dried circuit lines vs. the length of the circuit lines using a digital multi-meter (DVM890, Velleman). Then, the cross-sectional areas of the circuit lines were measured using a stylus profilometer (Dektak). Using the measured values for the cross sectional area (A) and the resistance (R) for a given length (L) of the circuit lines, the resistivity ( $\rho$ ) was calculated using the equation  $\rho = RA/L$ . Then the conductivity ( $\sigma$ ) was calculated by taking the reciprocal of the resistivity,  $\sigma = 1/\rho$ . The conductivity of this composition was measured to be 64,400 S/m.

For purposes of this detailed description, it is to be understood that the invention may assume various alternative variations and step sequences, except where expressly specified to the contrary. Moreover, other than in any operating examples, or where otherwise indicated, all numbers expressing, for example, quantities of ingredients used in the specification and claims are to be understood as being modified in all instances by the term "about". Accordingly, unless indicated to the contrary, the numerical parameters set forth in the following specification and attached claims are approximations that may vary depending upon the desired properties to be obtained by the present invention. At the very least, and not as an attempt to limit the application of the doctrine of equivalents to the scope of the claims, each numerical parameter should at least be construed in light of the number of reported significant digits and by applying ordinary rounding techniques.

Notwithstanding that the numerical ranges and parameters setting forth the broad scope of the invention are approximations, the numerical values set forth in the specific examples are reported as precisely as possible. Any numerical value, however, inherently contains certain errors necessarily resulting from the standard variation found in their respective testing measurements.

Also, it should be understood that any numerical range recited herein is intended to include all sub-ranges subsumed therein. For example, a range of "1 to 10" is intended to include all sub-ranges between (and including) the recited minimum value of 1 and the recited maximum value of 10, that is, having a minimum value equal to or greater than 1 and a maximum value of equal to or less than 10.

In this application, the use of the singular includes the plural and plural encompasses singular, unless specifically stated otherwise. In addition, in this application, the use of "or" means "and/or" unless specifically stated otherwise, even though "and/or" may be explicitly used in certain instances.

It will be readily appreciated by those skilled in the art that modifications may be made to the invention without

22

departing from the concepts disclosed in the foregoing description. Such modifications are to be considered as included within the following claims unless the claims, by their language, expressly state otherwise. Accordingly, the particular embodiments described in detail herein are illustrative only and are not limiting to the scope of the invention which is to be given the full breadth of the appended claims and any and all equivalents thereof.

10 We claim:

1. A resistive heating assembly comprising:  
a substrate;

a conductive coating applied to at least a portion of the substrate having a thickness of at least 1 micron comprising graphenic carbon particles dispersed in a polymeric film-forming resin binder throughout the thickness of the conductive coating, wherein the conductive coating has an electrical conductivity of greater than 10,000 S/m, and  
a source of electrical current connected to the conductive coating.

2. The resistive heating assembly of claim 1, wherein the conductive coating has a thickness of less than 100 microns.

3. The resistive heating assembly of claim 1, wherein the graphenic carbon particles comprise thermally produced graphenic carbon particles.

4. The resistive heating assembly of claim 3, wherein the thermally produced graphenic carbon particles have a BET specific surface area of at least 70 square meters per gram.

5. The resistive heating assembly of claim 1, wherein the graphenic carbon particles are functionalized.

6. A conductive coating having a thickness of from 1 to 100 microns and an electrical conductivity of greater than 10,000 S/m comprising graphenic carbon particles dispersed in a polymeric film-forming resin binder throughout the thickness of the conductive coating.

7. The conductive coating of claim 6, wherein the graphenic carbon particles comprise thermally produced graphenic carbon particles.

8. The conductive coating of claim 7, wherein the thermally produced graphenic carbon particles are produced in a thermal zone having a temperature of greater than 3,500° C. and have an average aspect ratio of greater than 3:1.

9. The conductive coating of claim 7, wherein the thermally produced graphenic carbon particles have a BET specific surface area of at least 70 square meters per gram.

10. The conductive coating of claim 6, wherein the graphenic carbon particles comprise at least two types of graphenic carbon particles.

11. The conductive coating of claim 10, wherein one of the types of graphenic carbon particles comprises thermally produced graphenic carbon particles.

12. The conductive coating of claim 11, wherein the thermally produced graphenic carbon particles comprise from 4 to 40 weight percent of the total amount of the graphenic carbon particles.

13. The conductive coating of claim 6, wherein the polymeric film-forming resin binder comprises epoxy resins, acrylic polymers, polyester polymers, polyurethane polymers, polyamide polymers, polyether polymers, bisphenol A based epoxy polymers, polysiloxane polymers, styrenes, ethylenes, butylenes, copolymers thereof, or combinations thereof.

14. The conductive coating of claim 6, wherein the graphenic carbon particles comprise from 40 to 95 weight percent of the conductive coating.

## 23

15. The conductive coating of claim 6, wherein the graphenic carbon particles comprise from 50 to 90 weight percent of the conductive coating.

16. The conductive coating of claim 6, wherein the electrical conductivity is greater than 20,000 S/m. 5

17. The conductive coating of claim 6, wherein the electrical conductivity is greater than 30,000 S/m.

18. The conductive coating of claim 6, wherein the coating is deposited from a co-dispersion comprising: 10  
a solvent;

at least one polymeric dispersant; and

at least two types of graphenic carbon particles co- 15  
dispersed in the solvent and the polymeric dispersant.

19. The resistive heating assembly of claim 1, wherein the conductive coating has a thickness of at least 5 microns.

20. The conductive coating of claim 6, wherein the conductive coating has a thickness of at least 5 microns. 15

21. A resistive heating assembly comprising:

a substrate;

a conductive coating applied to at least a portion of the 20  
substrate having a thickness of at least 1 micron comprising graphenic carbon particles dispersed in a poly-

## 24

meric film-forming resin binder throughout the thickness of the conductive coating wherein the conductive coating has an electrical conductivity of greater than 10,000 S/m; and

5 a source of electrical current connected to the conductive coating,

the graphenic carbon particles comprise thermally produced graphenic carbon particles and have a BET specific surface area of at least 70 square meters per gram.

22. A resistive heating assembly comprising:

a substrate;

a conductive coating applied to at least a portion of the substrate having a thickness of at least 1 micron comprising graphenic carbon particles dispersed in a poly- 15  
meric film-forming resin binder throughout the thickness of the conductive coating, wherein the graphenic carbon particles are functionalized; and

a source of electrical current connected to the conductive coating.

\* \* \* \* \*